

Aug. 19, 1969

C. H. G. BUSHELL ET AL  
PHOSPHATE FLOTATION PROCESS

3,462,016

Filed Aug. 28, 1967



INVENTOR.  
CHARLES H. G. BUSHELL  
HORST E. HIRSCH  
BY RANDOLPH M. LAUER

Arne J. Foss  
Agent

1

3,462,016

## PHOSPHATE FLOTATION PROCESS

Charles Herbert George Bushell, Montrose, British Columbia, Horst Eberhard Hirsch, Trail, British Columbia, and Randolph Mathias Lauer, Chapman Camp, British Columbia, Canada, assignors to Cominco Ltd., Montreal, Quebec, Canada, a company of Canada

Filed Aug. 28, 1967, Ser. No. 663,640

Claims priority, application Canada, Dec. 29, 1966,

979,171  
Int. Cl. B03d 1/00

U.S. Cl. 209—166

2 Claims

### ABSTRACT OF THE DISCLOSURE

A two-stage anionic flotation process for beneficiating phosphate-bearing materials containing calcium and magnesium carbonates and siliceous gangue material. In the first stage, the siliceous gangue material is selectively depressed and removed as underflow tailings while phosphate and carbonaceous materials are floated. The floated material is conditioned in an aqueous solution containing phosphoric acid and passed to the second flotation stage in which the carbonaceous material is floated and the phosphate minerals are recovered as an underflow concentrate.

This invention relates to a process for beneficiating phosphate-bearing materials and is particularly directed to an improved process for separating calcium and magnesium carbonates from phosphate minerals.

It is known to upgrade phosphate values in a phosphate-containing ore by means of flotation. One generally accepted process comprises suspending finely ground phosphate rock in a slightly alkaline aqueous solution containing a carboxylic acid or other anionic flotation reagent and subjecting the suspension to a first froth flotation step in which the phosphate values are concentrated and collected in the froth and a substantial portion of the siliceous gangue material is depressed and separated as the underflow tailing product. The concentrate from this first flotation step is then treated with sulphuric acid to remove the negative-ion collector reagent, filtered and washed with water to remove the residual sulphuric acid. The concentrate is then suspended in a neutral or substantially neutral aqueous solution containing an amine or other cationic flotation reagent and subjected to a froth flotation step in which the residual silica is collected in the froth and an enriched phosphate-containing concentrate is recovered as the underflow product.

A disadvantage of this process is the necessity for maintaining two separate and distinct flotation circuits, the first anionic and the second cationic, with the attendant problem of removing the flotation reagents from the concentrate from the anionic circuit before commencing treatment in the cationic circuit.

Another known process is that disclosed in U.S. Patent No. 3,113,838 issued Dec. 10, 1963. This patent describes a flotation process which employs a fatty acid in the presence of soluble alkaline phosphate produced by dissolving phosphate salt or by attacking a portion of the phosphate rock with a mineral acid such as sulphuric acid until phosphoric acid is freed, to transform calcium phosphate into a soluble phosphate. This acid addition is impractical when treating phosphate rock containing substantial amounts of silica as well as calcium and magnesium carbonates. In the presence of soluble phosphates there is no effective separation of phosphate minerals from silica and silicates.

2

Also, the treatment of a carbonate containing ore with a strong mineral acid, such as sulphuric acid, would require the addition of an excessive amount of acid due to the preferential attack on the carbonates, and would unfavorably alter the characteristics of the feed to the flotation operation.

It is important for the production of a phosphate concentrate suitable for use in the wet phosphoric acid process that carbonate containing minerals, especially magnesium-containing carbonates, be maintained at a minimum. The presence of carbonates not only causes undesirable foaming in the reactor chambers and undue consumption of acids, but also the magnesium content in the carbonates forms a magnesium sulphate which is soluble in phosphoric acid producing a magnesium salt upon subsequent ammoniation of the phosphoric acid which lowers the value of the ammonium phosphate fertilizer product. Also, the presence of magnesium in the phosphoric acid raises the viscosity of the salt.

20 We have discovered that a phosphate concentrate produced from a conventional first stage anionic flotation circuit which has been conditioned in the presence of a small amount of phosphoric acid in an aqueous solution to produce a pH of from 4.5 to 5.8 can be passed to a second stage anionic flotation circuit, with or without additional amounts of the same flotation reagents as those used in the first stage, to provide an effective separation and removal of the phosphate minerals from the non-phosphate gangue minerals, especially the deleterious calcium and magnesium carbonate minerals.

25 It is a principal object of the present invention, therefore, to provide a two-stage anionic flotation circuit for beneficiating phosphate-bearing materials which obviates the necessity of neutralizing or destroying the flotation reagents used in a first stage anionic flotation circuit prior to reflootation treatment of the concentrate from the first stage.

Another object of the present invention is the removal of a major portion of residual calcium and magnesium carbonate minerals present in a phosphate mineral concentrate made from a siliceous ore.

30 And another object of the invention is the provision of a process which permits utilization, and recovery for re-use, of an inexpensive conditioning agent.

35 These and other objects of the invention and the manner in which they can be attained will become apparent from the following description of the process as illustrated in the drawing in which:

The drawing provides a schematic illustration of a flowsheet showing the process steps of an embodiment of the invention.

According to the process of the invention, the phosphate rock to be beneficiated preferably is subjected, after appropriate comminution, to a primary anionic flotation stage, using fatty acid collector reagents such as oleic acid, stearic acid, or other carboxylic acids, including tall oils and the like, to provide an enriched phosphate concentrate containing calcium and magnesium carbonates as a froth product and a silica tailing as an underflow depressed product. Phosphate rocks, containing such minerals as collophane, are first comminuted for liberation of the phosphate minerals from the gangue minerals. The degree of grinding applied to the rock will depend, of course, on the texture of the rock and association of the phosphate values with the gangue minerals.

With reference to the flowsheet of the drawing, it will be seen that the phosphate rock is comminuted to the desired size range necessary to liberate the phosphate values from the gangue by crushing and grinding steps 40 and 12 respectively and classified in classifiers 14 to yield a sized product which is suspended in water or

recycled solution and conditioned in stage 16 by the addition of carboxylic acid, sodium silicate and an alkali for a pH of 9 to 10.5. The conditioned material is subjected to a first stage flotation 18 in an anionic circuit for production of a phosphate-enriched float concentrate and a siliceous gangue underflow. The gangue normally is thickened in stage 20 and discharged to waste. The primary separation of phosphate minerals from siliceous gangue minerals as described above is well known in the art.

The phosphate-enriched float concentrate is then thickened in a thickener or hydroclone stage 22 and passed to a conditioner 24 having an aqueous solution therein maintained at a pH in the range of from about 4.5 to 5.8 by the controlled addition of phosphoric acid. The conditioned slurry, to which is added carboxylic acid, is then passed to a second stage anionic flotation circuit 26 for production of an overflow product of gangue material, especially calcium and magnesium carbonate minerals, and an underflow product of phosphate-enriched concentrate which is thickened in stage 28 and the thickener underflow filtered in unit 30 for the production of a phosphate concentrate. The float product from the flota-

The concentrate from the first stage separation was pumped to a thickener and the thickener underflow containing approximately 65% solids was pumped to a conditioning tank and the following reagents were added:

5 Phosphoric acid, ( $H_3PO_4$ ), 3-8 lbs. per ton of first stage concentrate to produce pH 4.5 to 5.8 when diluted as described below.

Tall oil (fatty acid), 0 to 3 lbs. per ton of first stage concentrate.

10 This suspension was then diluted with water to contain 30 to 35% solids by weight and fed to a flotation machine.

Table 1 below gives the analysis, weight and percent distribution of the  $P_2O_5$ , CaO, MgO and  $SiO_2$  contained in the feed, concentrate and tailing produced in the first stage separation.

15 Table 2 gives the analysis, weight and percent distribution of the  $P_2O_5$ , CaO, MgO and  $SiO_2$  contained in the concentrate and tailing produced in the second stage separation.

20 Table 3 provides a comparison of the first stage recoveries relative to the overall recoveries of the process.

TABLE 1.—FIRST STAGE SEPARATION

|                        | Composition (percent) |      |      |        |         | Wt. | Distribution (percent) |      |      |        |         |
|------------------------|-----------------------|------|------|--------|---------|-----|------------------------|------|------|--------|---------|
|                        | $P_2O_5$              | CaO  | MgO  | $CO_2$ | $SiO_2$ |     | $P_2O_5$               | CaO  | MgO  | $CO_2$ | $SiO_2$ |
| Feed                   | 20.2                  | 31.5 | 0.9  | 3.5    | 28.5    | 100 | 100                    | 100  | 100  | 100    | 100     |
| Concentrate (overflow) | 30.6                  | 45.1 | 1.17 | 5.3    | 10.5    | 58  | 87.9                   | 83.0 | 75.4 | 87.8   | 21.4    |
| Tailings (underflow)   | 5.8                   | 12.7 | 0.53 | 1.0    | 53.4    | 42  | 12.1                   | 17.0 | 24.6 | 12.2   | 78.6    |

TABLE 2.—SECOND STAGE SEPARATION

|                         | Composition (percent) |      |      |        |         | Wt.  | Distribution (percent) |      |      |        |         |
|-------------------------|-----------------------|------|------|--------|---------|------|------------------------|------|------|--------|---------|
|                         | $P_2O_5$              | CaO  | MgO  | $CO_2$ | $SiO_2$ |      | $P_2O_5$               | CaO  | MgO  | $CO_2$ | $SiO_2$ |
| Feed                    | 30.6                  | 45.1 | 1.17 | 5.3    | 10.5    | 100  | 100                    | 100  | 100  | 100    | 100     |
| Concentrate (underflow) | 32.1                  | 46.1 | 0.50 | 3.7    | 10.7    | 90.8 | 95.2                   | 92.8 | 38.8 | 63.4   | 92.5    |
| Tailings (overflow)     | 15.8                  | 35.2 | 7.78 | 21.1   | 8.5     | 9.2  | 4.8                    | 7.2  | 61.2 | 36.6   | 7.5     |

tion circuit 26 normally is also thickened in unit 32 and the thickener underflow discharged to waste. The solutions recovered from units 28, 30 and 32 can be discharged to waste or re-cycled to conditioner 24 for utilization of the reagents therein.

It will be understood that the addition of flotation reagents such as carboxylic acid and the like may not be necessary due to the presence of flotation reagents retained from the first stage anionic circuit. The rate of addition of phosphoric acid for conditioning the feed to the second stage is primarily determined by the pH of the aqueous solution. We have found that optimum results are attained with a pH within the range of from about 4.5 to about 5.8. With different ores, however, this optimum pH range may vary somewhat, for example, from about pH 4 to about pH 6. The effectiveness of the separation of calcium and magnesium carbonates from the phosphates in the second stage anionic flotation circuit is reduced with solution pH's outside this range of about 4 to 6.

The following examples show the effectiveness of the present process in the treatment of a colophane phosphate rock indigenous to the Western United States.

#### EXAMPLE 1

In this example of the process of our invention a phosphate rock was ground to 60-80% minus 200 mesh and suspended in an aqueous solution having a pH of 9 to 10.5 and containing the following reagents:

|                  | Lbs. per ton of ore |
|------------------|---------------------|
| Fatty acid       | 1.5                 |
| Sodium hydroxide | 3.0                 |
| Sodium silicate  | 1.0                 |

The liquid-solids ratio of this suspension was adjusted to 30 to 35% solids by weight and the suspension was fed to a flotation machine.

40

45

TABLE 3.—RECOVERIES (PERCENT)

|         | $P_2O_5$ | CaO  | MgO  | $CO_2$ | $SiO_2$ |
|---------|----------|------|------|--------|---------|
| First   | 87.9     | 88.0 | 75.4 | 87.8   | 21.4    |
| Overall | 83.7     | 77.0 | 29.3 | 55.7   | 10.8    |

50 It will be noted from the above tables that 95.2% of the  $P_2O_5$  contained in the feed to the second stage flotation was recovered in the flotation machine underflow and that 61.2% of the MgO was rejected in the overflow; the overall recovery of  $P_2O_5$  being 83.7% and the overall recovery of MgO being 29.3%. The effective reduction of MgO in the concentrate relative to the feed 55 was therefore  $(100 - 29.3) = 70.7\%$ .

#### EXAMPLE 2

In this example of the process an ore comminuted as described above was treated according to the conditions set forth in Example 1.

Tables 4, 5 and 6 below provide data for the first stage separation, second stage separation and recoveries of the first stage relative to the first and second stages combined respectively, as was described hereinabove with reference to Tables 1, 2 and 3. It will be noted that 94.7% of the  $P_2O_5$  contained in the feed to the second stage flotation was recovered in the flotation machine underflow and that 67.1% of the MgO was rejected in the overflow; the overall recovery of  $P_2O_5$  being 80.3% and the overall recovery of MgO being 27.0%. The effective reduction of MgO in the concentrate relative to the feed 75 was therefore  $(100 - 27.0) = 73.0\%$ .

TABLE 4.—FIRST STAGE SEPARATION

|                             | Composition (percent)         |      |      |                 |                  | Wt. | Distribution (percent)        |      |      |                 |                  |
|-----------------------------|-------------------------------|------|------|-----------------|------------------|-----|-------------------------------|------|------|-----------------|------------------|
|                             | P <sub>2</sub> O <sub>5</sub> | CaO  | MgO  | CO <sub>2</sub> | SiO <sub>2</sub> |     | P <sub>2</sub> O <sub>5</sub> | CaO  | MgO  | CO <sub>2</sub> | SiO <sub>2</sub> |
| Feed.....                   | 19.8                          | 30.8 | 1.1  | 3.7             | 29.1             | 100 | 100                           | 100  | 100  | 100             | 100              |
| Concentrate (overflow)..... | 30.0                          | 45.0 | 1.63 | 6.0             | 10.5             | 56  | 84.8                          | 81.8 | 83.0 | 90.8            | 20.2             |
| Tailings (underflow).....   | 6.8                           | 12.7 | 0.43 | 0.8             | 52.8             | 44  | 15.2                          | 18.2 | 17.0 | 9.2             | 79.8             |

TABLE 5.—SECOND STAGE SEPARATION

|                              | Composition (percent)         |      |      |                 |                  | Wt.  | Distribution (percent)        |      |      |                 |                  |
|------------------------------|-------------------------------|------|------|-----------------|------------------|------|-------------------------------|------|------|-----------------|------------------|
|                              | P <sub>2</sub> O <sub>5</sub> | CaO  | MgO  | CO <sub>2</sub> | SiO <sub>2</sub> |      | P <sub>2</sub> O <sub>5</sub> | CaO  | MgO  | CO <sub>2</sub> | SiO <sub>2</sub> |
| Feed.....                    | 30.0                          | 45.0 | 1.63 | 6.0             | 10.5             | 100  | 100                           | 100  | 100  | 100             | 100              |
| Concentrate (underflow)..... | 32.1                          | 45.6 | 0.60 | 3.6             | 10.5             | 88.6 | 94.7                          | 89.8 | 32.5 | 52.9            | 89.4             |
| Tailings (overflow).....     | 13.7                          | 40.4 | 9.63 | 24.6            | 9.7              | 11.4 | 5.3                           | 10.2 | 67.5 | 47.1            | 10.6             |

TABLE 6.—RECOVERIES (PERCENT)

|                             | P <sub>2</sub> O <sub>5</sub> | CaO  | MgO  | CO <sub>2</sub> | SiO <sub>2</sub> |
|-----------------------------|-------------------------------|------|------|-----------------|------------------|
| First stage recoveries..... | 84.8                          | 81.8 | 83.0 | 90.8            | 20.2             |
| Overall recoveries.....     | 80.3                          | 73.5 | 27.0 | 48.0            | 18.1             |

Although it will be understood that the present invention is free from hypothetical considerations, it is believed that the improvement in the present process, the separation of a major portion of the residual calcium and magnesium carbonates from the phosphate concentrates in the second stage of a two-stage anionic circuit, results from the addition of a small amount of phosphoric acid to the feed for the second stage. It is not definitely ascertained why the addition of phosphoric acid to the feed to the second stage should result in the depression of the phosphate particles and the flotation of the residual gangue material, which is contrary to what occurs in the first stage separation in which the phosphate particles float and the silica gangue is depressed. The lowering of the pH by the addition of sulphuric acid or other acids is not sufficient, per se, in bringing about the improvement of the present invention. It appears that the presence of a phosphate ion may be instrumental in affecting the flotation characteristics of the phosphate mineral possibly because of its effect on the solubility relationships of the phosphate particles and gangue particles in the suspension.

The present invention provides a number of important advantages. Phosphate-bearing materials can be beneficiated by the removal of gangue materials such as calcium and magnesium carbonates in a two-stage anionic flotation circuit by the simple expedient of adding phosphoric acid, a product from the wet phosphoric acid process to which the phosphate concentrate is subsequently subjected, to the concentrate from the first stage flotation. The reagents from the first stage need not be destroyed and can often provide the necessary concentration of reagents to effect the subsequent flotation operation in the second stage.

What we claim as new and desire to protect by Letters Patent of the United States is:

1. A process for beneficiating a siliceous phosphate rock high in calcium carbonate and magnesium carbonate comminuted for the substantial liberation of phosphate values from silica, calcium carbonate and magnesium carbonate by froth flotation which comprises the steps of subjecting said phosphate rock in finely-divided form to a primary anionic flotation, separately withdrawing from said primary flotation an underflow tailings product high in silica content and a phosphate-enriched float product containing calcium carbonate and magnesium carbonate, conditioning said phosphate-enriched float product in an aqueous solution having phosphoric acid added thereto in amount sufficient to maintain a pH within the range of from about 4.5 to about 5.8, subjecting said conditioned float product to a secondary anionic flotation and separately withdrawing from said secondary flotation a float product high in calcium carbonate and magnesium carbonate and an underflow concentrate product high in phosphate-bearing minerals.

2. In a process as claimed in claim 1, recovering the aqueous solution having phosphoric acid added thereto and recycling said solution to the conditioning step.

#### References Cited

##### UNITED STATES PATENTS

|    |           |         |           |           |
|----|-----------|---------|-----------|-----------|
| 45 | 2,442,455 | 6/1948  | Booth     | 209—166   |
|    | 3,032,197 | 5/1962  | Northcott | 209—166   |
|    | 3,113,838 | 12/1963 | Perri     | 209—166 X |
|    | 3,259,242 | 7/1966  | Snow      | 209—166   |

##### FOREIGN PATENTS

|    |         |        |         |
|----|---------|--------|---------|
| 50 | 468,161 | 9/1950 | Canada. |
|----|---------|--------|---------|

HARRY B. THORNTON, Primary Examiner

R. HALPER, Assistant Examiner